

Patented Feb. 20, 1923.

1,446,153

# UNITED STATES PATENT OFFICE.

WILLIAM B. BROOKFIELD, OF SYRACUSE, NEW YORK.

## METHOD OF MAKING HIGH-SPEED STEEL.

No Drawing.

Application filed December 29, 1920. Serial No. 433,775.

To all whom it may concern:

Be it known that I, WILLIAM B. BROOKFIELD, of Syracuse, in the county of Onondaga, in the State of New York, have invented new and useful Improvements in Methods of Making High-Speed Steel, of which the following, taken in connection with the accompanying drawings, is a full, clear, and exact description.

10 This invention relates to an improved method or process of producing "high speed" steel involving not only the use of certain selected materials or ingredient elements in suitable proportions, known to those skilled in this art and not necessary to herein describe, but also involving the heat treatment of those materials "en masse" during the melting period in such manner as to combine them into a unitary homogeneous mass which, when cast into ingots or pigs or worked into cutting tools and other implements, will retain substantially the same degree of homogeneity and other desired characteristics.

25 The methods heretofore employed in the manufacture of this grade of steel consisted in subjecting the ingredient elements to a single continuous melting heat, either in an electric furnace or in a series of separate crucibles, but in each case it is found that even with the exercise of the utmost care and skill in the manipulation of the heat during the melting period, the materials tend to stratify according to their various specific gravities and that the reluctance to assimilation, particularly of the heavier strata, introduces a factor of unreliability in the degree of homogeneity and resultant defects in the product.

35 40 These defects are often not discernible in the broken pigs or ingots and in many instances do not appear until the product is worked into cutting tools and other implements and then only when the tool is actually used and broken by reason of the defect in the performance of some work all of which entails a considerable loss and accounts, in a measure, for the present high cost of production.

45 50 These breakages are in most instances the result of imperceptibly fine hair-like cleavages in the material from which the tool is made, due to imperfect homogenization of the materials in the molten mass before being cast into the pigs or ingots and ap-

parently cannot be avoided by the single melting process, but after repeated experiments over a considerable period of time, I have discovered that these defects may, almost entirely, be overcome and the homogeneity of the product greatly increased by subjecting the ingredient materials to successive melting heats, preferably as follows:

That is, the materials necessary to the production of "high speed" steel are first reduced "en masse" to a molten state in an electric furnace under a temperature sufficient to produce a maximum assimilation and homogeneity under that temperature, which is usually as high as any known lining will withstand, after which the product is drawn off and cast into suitable ingots or pigs.

In order to complete the process of homogenization these ingots or pigs are broken in fragments and resubjected to a melting heat, preferably in a series of crucibles, and under a lesser degree of heat than that employed in the first melting with the result that the granules of the various materials are brought into more closely commingling relation or greater homogeneity which in turn produces a better grade of tool and eliminates practically all of the wastage incident to the previous processes.

While the foregoing method is preferable, it may be possible to obtain equally beneficial results by withdrawing the molten metal from the first electric furnace directly into one or more additional electric furnaces, or directly into the crucibles, and resubjecting it to another melting heat of the same or lower temperature without departing from the spirit of this invention which consists primarily in subjecting the same materials to at least two melting heats or periods.

What I claim is:

1. The herein described method of making "high speed" steel, consisting in subjecting the ingredient element "en masse" to continuous heat sufficient to produce a maximum degree of homogeneity under that heat and afterward resubjecting the product thus formed to another melting heat sufficient to cause a further and more uniform assimilation of said ingredient elements and, therefore, to increase the homogeneity without the addition of other materials.

2. The herein described method of making "high speed" steel, as in claim 1, in

which the melting heat in the second treatment is of lesser degree than that of the first melting heat.

3. The herein described method of making "high speed" steel, as in claim 1, in which the first reduction of the ingredients to its molten state is produced in an electric furnace.

4. The herein described method of making "high speed" steel, as in claim 1, in which the retreatment of the first named product is carried out in crucibles.

5. The herein described method of making "high speed" steel, as in claim 1, in which the materials are first treated in an electric furnace and the product thus produced afterward treated in crucibles.

6. The herein described method of making "high speed" steel, consisting in subjecting the ingredient elements "en masse" to continuous heat sufficient to produce a maximum degree of homogeneity under that heat, then casting the product thus produced into ingots or pigs and subsequently reducing the ingots or pigs to a molten state under a lesser degree of heat than that employed in the first reduction.

7. The herein described method of making "high speed" steel, consisting in subjecting the ingredient elements "en masse" to continuous heat sufficient to produce a

maximum degree of homogeneity under that heat, then casting the product thus formed into ingots or pigs and afterward retreating the ingots or pigs in crucibles.

35

8. The herein described method of making "high speed" steel, consisting in melting the ingredient elements "en masse" in an electric furnace under a continuous heat sufficient to produce a maximum degree of homogeneity under that heat, then casting the product thus produced into ingots or pigs and afterward remelting the ingots or pigs in crucibles.

40

9. The herein described method of making "high speed" steel, consisting in melting the ingredient elements "en masse" in an electric furnace under a continuous heat sufficient to produce a maximum degree of homogeneity under that heat, then casting the product thus produced into ingots or pigs and afterward breaking the ingots or pigs into fragments and remelting the fragments in crucibles under a lesser degree of heat than that to which the ingredients were subjected in the electric furnace.

45

In witness whereof I have hereunto set my hand this 15th day of December, 1920.

WILLIAM B. BROOKFIELD.

Witnesses:

H. E. CHASE,

M. R. COOKE.